

Dec. 6, 1966

G. A. OAKES

3,289,292

BUILT-UP STRIP MILL GUIDE

Filed Oct. 29, 1964

FIG. 1



FIG. 2



FIG. 3



FIG. 4



FIG. 5

INVENTOR  
GRANT A. OAKES

BY *W.B. Harpman*

ATTORNEY



of the guide 10 to form bubbles in the deposited molten metal which quickly solidifies and traps the bubbles in random orientation therein.

The relatively harder metal 21 is deposited by filling up the groove 16 progressively in one pass of the torch 18 through which the spooled wire W is continuously fed and thereby melted and deposited.

In a typical arrangement the heat from the torch nozzle 19 will flow back over the deposited metal 21 toward the left in FIGURE 2 to form a smooth closed surface thereon. The temperature of the torch is related to the speed of the wire which is generally 2'-3' per second. The torch 18 is moved at an average rate of about 4' per second. This procedure will result in a perfect bond between the relatively harder metal 21 and the relatively softer metal of the strip metal guide body 10. When the groove 16 has been completely filled from one end to the other, as it appears in cross section in FIGURE 4 of the drawings with the bubbles 22 therein, the strip mill guide body is cooled, preferably with air although a water quench can be used, and the excess metal as appears in FIGURE 4 of the drawings is then ground off, or otherwise removed, to form the transversely flat surface as it appears in FIGURES 1 and 5 of the drawings. The illustration in FIGURE 5 of the drawings shows the deposited relatively harder metal 21 positioned in the groove 16 of the strip metal guide body 10 where it has bonded completely therewith and the top surface has been removed, as hereinbefore referred to, to form the uniformly transversely flat surface.

The next step in the formation of the built-up strip metal guide is to straighten the same so as to overcome the arc which normally occurs during the preheating and welding in of the relatively hard metal 21. When the straightening has been completed, the build-up rolling mill guide appears as in FIGURE 1 of the drawings, and it is then ready for installation in a strip mill where it will considerably outlast the rolling mill guides heretofore known in the art.

Those skilled in the art will recognize that such rolling mill guides as heretofore known in the art are generally formed of a copper base alloy, such as bearing bronze, or the like. The relatively harder metal which is used to build up the desirable wearing surface longitudinally of and centrally of the strip mill guide body is considerably harder than the bearing bronze of which the strip mill guide body 10 is formed, and at the same time it is relatively softer than the steel strip which is guided thereby so that it is entirely suitable for the purpose intended.

It will thus be seen that a built-up strip mill guide has been disclosed, together with the method of making the same, which produces a superior article and which may, incidentally, be produced by reworking used worn-out strip mill guides.

It will occur to those skilled in the art that the longitudinal center line built-up area of the strip mill guide body as disclosed herein is in the desirable position to

receive a majority of the wear resulting from contact by the lateral edges of the strip material, such as strip steel being guided. It will also occur to those skilled in the art that the deflection of the strip material being guided will cause the same to properly enter the stands of rolls of the strip mill, while at the same time presenting suitable wearing surfaces capable of relatively long life.

It will be seen that the formation of the metal 21 in the strip mill guide body 10 with the bubbles 22 therein provides a series of desirably located grease and/or oil traps which fill with lubricant applied to the guide or to the edges of the traveling strip and continue to supply the lubricant as needed. The combination of these built-in lubricant pockets and the desirable welded in metal 21 result in the greatly extended life of the guides so formed.

The built-up strip mill guide disclosed herein has been described in connection with a continuous strip mill and a stand of rolls therein, and it will occur to those skilled in the art that the guides might equally well be applied to similar metal strip handling, working, and fabricating operations where it is desired to guide a traveling strip in a fixed path, and having thus described my invention, what I claim is:

1. The method of making a guide for traveling strip in a strip mill and the like that comprises forming an elongated groove in an elongated metallic body member, heating said member to a temperature between 900° and 1200° F. and depositing a groove filling body of molten metal of the group including silicon bronze alloy and Phosphor bronze alloy in said groove at a temperature sufficient to vaporize some of the metal of said body member and trap the same in said molten metal so as to form bubbles therein, cooling said body member, removing metal to form a transversely flat wearing surface and straightening said body member so that it is longitudinally flat.

2. The method of making a guide set forth in claim 1 and wherein said metal deposited in said groove is melted by a metal insert gas process torch arranged to form a heat cover.

#### References Cited by the Examiner

#### UNITED STATES PATENTS

|           |         |                |       |        |
|-----------|---------|----------------|-------|--------|
| 1,255,469 | 2/1918  | Schlieder      | ----- | 29—481 |
| 1,956,462 | 4/1934  | Knuth          | ----- | 29—529 |
| 1,999,599 | 4/1935  | Smith          | ----- | 29—529 |
| 2,185,657 | 1/1940  | Brangle et al. | ----- | 72—428 |
| 2,241,789 | 5/1941  | Queneau et al. | ----- | 29—529 |
| 2,250,561 | 7/1941  | Wissler        | ----- | 29—529 |
| 2,258,913 | 10/1941 | Stone          | ----- | 29—481 |

55 CHARLES W. LANHAM, *Primary Examiner.*

H. D. HOINKES, *Assistant Examiner.*